



US010359716B2

(12) **United States Patent**  
**Sato**

(10) **Patent No.:** US 10,359,716 B2  
(45) **Date of Patent:** Jul. 23, 2019

(54) **IMAGE FORMING UNIT AND IMAGE FORMING APPARATUS**

(71) Applicant: **Oki Data Corporation**, Tokyo (JP)

(72) Inventor: **Toshiharu Sato**, Tokyo (JP)

(73) Assignee: **Oki Data Corporation**, Tokyo (JP)

(\*) Notice: Subject to any disclaimer, the term of this patent is extended or adjusted under 35 U.S.C. 154(b) by 0 days.

(21) Appl. No.: **16/010,901**

(22) Filed: **Jun. 18, 2018**

(65) **Prior Publication Data**

US 2018/0373178 A1 Dec. 27, 2018

(30) **Foreign Application Priority Data**

Jun. 26, 2017 (JP) ..... 2017-123819

(51) **Int. Cl.**

**G03G 15/08** (2006.01)

(52) **U.S. Cl.**

CPC . **G03G 15/0808** (2013.01); **G03G 2215/0641** (2013.01)

(58) **Field of Classification Search**

USPC ..... 399/252, 279, 281, 286

See application file for complete search history.

(56) **References Cited**

U.S. PATENT DOCUMENTS

9,046,818 B2 \* 6/2015 Sato ..... G03G 15/0808

FOREIGN PATENT DOCUMENTS

JP 2005-148664 A 6/2005

\* cited by examiner

*Primary Examiner* — Hoan H Tran

(74) *Attorney, Agent, or Firm* — Metrolexis Law Group, PLLC

(57) **ABSTRACT**

A developer supply member according to an embodiment includes: a shaft with conductivity; and a conductive foam layer that is formed on a surface of the shaft. The conductive foam layer contains silicone rubber as a main component and includes a stress decay of 25% or less and a residual strain of 100  $\mu$ m or less.

**17 Claims, 10 Drawing Sheets**





FIG. 2



FIG. 3



FIG. 4A



FIG. 5



FIG. 6



FIG. 7



FIG. 8



FIG. 9



FIG. 10



## IMAGE FORMING UNIT AND IMAGE FORMING APPARATUS

### CROSS REFERENCE TO RELATED APPLICATIONS

This application claims priority based on 35 USC 119 from prior Japanese Patent Application No. JP2017-123819 filed on Jun. 26, 2017, entitled "IMAGE FORMING UNIT AND IMAGE FORMING APPARATUS", the entire contents of which are incorporated herein by reference.

### BACKGROUND

The disclosure relates to an image forming apparatus such as a printer, a copy machine, and a facsimile, and an image forming unit used for the image forming apparatus.

In an image forming apparatus using the electrophotography, an electrostatic latent image is formed on the surface of a photoconductor drum, and is developed by a developer held on the surface of a developing roller. The developer is supplied to the developing roller by a supply roller. The supply roller is a roller (such as a sponge roller) in which a conductive foam layer is formed on the surface of a shaft made of metal or the like. The supply roller is disposed to be in contact with the surface of the developing roller.

Related techniques are disclosed in, for example, Japanese Unexamined Patent Application Publication No. 2005-148664.

### SUMMARY

When the conductive foam layer of the supply roller is left unoperated for a long period of time in contact with the developing roller, a depressed area may be formed in the contact portion with the developing roller. With such a depressed area formed in the conductive foam layer, when image formation is resumed, the developer is not sufficiently supplied to the developing roller at a portion corresponding to the depressed area, resulting in a problem in that a belt of an uneven image occurs.

An object of an embodiment is to reduce the occurrence of image unevenness which is caused by the conductive foam layer, and to improve image quality.

An aspect is a developer supply member that includes: a shaft with conductivity; and a conductive foam layer that is formed on a surface of the shaft. The conductive foam layer contains silicone rubber as a main component and includes a stress decay of 25% or less and a residual strain of 100  $\mu\text{m}$  or less.

Another aspect is an image forming unit that includes: a developer carrier that supplies a developer to an image carrier with a surface on which a latent image is formed, and that develops the latent image; and a developer supply member disposed in contact with the developer carrier. The developer supply member includes: a shaft with conductivity; and a conductive foam layer that is formed on a surface of the shaft. The conductive foam layer contains silicone rubber as a main component and includes a stress decay of 25% or less and a residual strain of 100  $\mu\text{m}$  or less.

According to the aspects, deformation of an elastic foam layer can be suppressed and image quality can be improved.

### BRIEF DESCRIPTION OF DRAWINGS

FIG. 1 is a diagram illustrating the configuration of an image forming apparatus in an embodiment;

FIG. 2 is a cross-sectional view illustrating the configuration of an image forming unit in an embodiment;

FIG. 3 is a block diagram illustrating the principal unit of a control system of the image forming apparatus;

FIGS. 4A and 4B are a front view and a cross-sectional view illustrating the supply roller in an embodiment;

FIG. 5 is a flowchart for explaining the manufacturing process of the supply roller;

FIG. 6 is a temperature rise curve in a vulcanization step for a conductive foam layer in the manufacturing process of the supply roller;

FIG. 7 is a schematic illustration for explaining a method of measuring stress decay and residual strain of the supply roller;

FIG. 8 is a graph illustrating the hysteresis loop in measurement of FIG. 7;

FIG. 9 is a schematic illustration depicting an example of image unevenness; and

FIG. 10 is a flowchart illustrating a modification of the manufacturing process of the supply roller.

### DETAILED DESCRIPTION

Descriptions are provided hereinbelow for embodiments based on the drawings. In the respective drawings referenced herein, the same constituents are designated by the same reference numerals and duplicate explanation concerning the same constituents is omitted. All of the drawings are provided to illustrate the respective examples only.

#### <Configuration of Image Forming Apparatus>

FIG. 1 is a diagram illustrating the basic configuration of an image forming apparatus 1 in one or more embodiments. The image forming apparatus 1 is configured as a color electrophotographic printer here. The image forming apparatus 1 includes image forming units 2K, 2C, 2M, and 2Y that form toner images of black (K), cyan (C), magenta (M), and yellow (Y), respectively; LED heads 5K, 5C, 5M, and 5Y that irradiate respective photoconductor drums (described below) of the image forming units 2K, 2C, 2M, and 2Y with light; a transfer unit 4 that transfers the toner images onto paper P; and a fixing unit 7 that fixes the toner images to the paper P.

The image forming apparatus 1 also includes a paper feed cassette 60 that stores the paper P (medium); a pickup roller 61 that delivers the paper P stored in the paper feed cassette 60 to a transport path 8; a transport roller pair 62 that transports the paper P delivered to the transport path 8 to the image forming units 2K, 2C, 2M, and 2Y; and a discharge roller pair 63 that discharges the paper P which has passed through the fixing unit 7.

The paper feed cassette 60 (medium storage) stores sheets of the paper P as media with the sheets stacked, and is detachably mounted in a lower portion of the image forming apparatus 1.

The pickup roller 61 feeds the sheets of the paper P stored in the paper feed cassette 60 one by one, and delivers the paper P to the transport path 8 as indicated by an arrow A. The transport roller pair 62 corrects skew of the paper P delivered to the transport path 8 by the pickup roller 61, and transports the paper P to the image forming units 2K, 2C, 2M, and 2Y as indicated by an arrow B.

The image forming units 2K, 2C, 2M, and 2Y form toner images of black, cyan, magenta, and yellow, and are arranged in a row (here, from the right to the left in FIG. 1) along the transport path 8 of the paper P. Also, the image forming units 2K, 2C, 2M, and 2Y are detachably mounted in the image forming apparatus 1.

FIG. 2 is a cross-sectional view illustrating the configuration of the image forming units 2. The image forming units 2K, 2C, 2M, and 2Y have a common configuration except for each toner (developer) to be used. Therefore, the image forming units 2K, 2C, 2M, and 2Y and their components will be described with the symbols K, C, M, and Y omitted.

As illustrated in FIG. 2, the image forming units 2 have respective photoconductor drums 21 as image carriers. The photoconductor drums 21 rotate in the direction indicated by an arrow R in FIG. 2. A charging roller 22 as a charging member, a developing roller 23 as a developer carrier, and a cleaning blade 26 as a cleaning member are disposed around each of the photoconductor drums 21 in a rotational direction.

Also, a supply roller 25 as a supply member, and a developing blade 24 as a layer regulation member are disposed around the developing roller 23. A toner storage chamber 20a, which is space for storing toner, is formed above the supply roller 25 and the developing blade 24. The axial direction of each roller of the image forming units 2 and the longitudinal direction of the developing blade 24 are parallel to the axial direction of the photoconductor drum 21.

Although stirring members 28a, 28b, and 28c that stir toner, and a transport screw 29 for uniformly leveling the toner in the axial direction are disposed in the toner storage chamber 20a, a description of these is omitted.

A toner cartridge 3 (developer storage body) for supplying toner is mounted in each image forming unit 2. The toner cartridge 3 is detachably mounted, for instance, in an upper portion of the body of the image forming unit 2.

The toner cartridge 3 has a toner storage 31 that stores toner, and has a stirring bar 32 that stirs toner, inside the toner storage 31. Also, a toner supply port 33 for supplying toner to the toner storage chamber 20a of the image forming unit 2 is formed at the bottom of the toner cartridge 3.

The photoconductor drum 21 has a cylindrical conductive support 21b, and a photoconductive layer 21a formed on the surface of the conductive support 21b. The conductive support 21b is made of, for instance, a metal pipe such as an aluminum pipe. The photoconductive layer 21a includes a laminated body of a charge generation layer and a charge transport layer. A blocking layer (intermediate layer) may be provided between the conductive support 21b and the photoconductive layer 21a.

The charging roller 22 is provided so as to be in contact with the surface of the photoconductor drum 21, and follows the rotation of the photoconductor drum 21 and rotates. The charging roller 22 has, for instance, a shaft 22b made of metal, and an elastic layer 22a formed on the surface of the shaft 22b. The elastic layer 22a is a semiconductive rubber layer made of, for instance, semiconductive epichlorohydrin rubber.

The developing roller 23 is disposed so as to be in contact with the surface of the photoconductor drum 21. Also, the developing roller 23 rotates in the direction opposite to the rotational direction of the photoconductor drum 21 (in other words, in the same direction of movement at the contact portion on the surface) at a predetermined circumferential speed ratio. The developing roller 23 has, for instance, a shaft 23b made of metal such as stainless steel, and an elastic layer 23a formed on the surface of the shaft 23b. The elastic layer 23a is made of, for instance, semiconductive urethane rubber. A surface treatment layer may be provided on the surface of the elastic layer 23a.

The developing blade 24 is a metal plate-shaped member having substantially the same length as the axial length of the elastic layer 23a of the developing roller 23. The

thickness of the developing blade 24 is, for instance, 0.08 mm. The developing blade 24 has one end fixed to a frame 20 of the image forming unit 2 and a bent portion formed on the other end side in pressure contact with the surface of the developing roller 23. The developing blade 24 regulates the thickness of a toner layer formed on the surface of the developing roller 23.

The supply roller 25 is disposed so as to be in contact with the surface of the developing roller 23. Also, the supply roller 25 rotates in the same direction as the rotational direction of the developing roller 23 (in other words, in the direction opposite to the direction of movement at the contact portion on the surface) at a predetermined circumferential speed ratio. The supply roller 25 has a shaft 25b made of, for instance, metal, and a conductive foam layer 25a (silicone sponge layer) provided on the surface of the shaft 25b.

The cleaning blade 26 is made of, for instance, urethane rubber, and is disposed so as to be in contact with the surface of the photoconductor drum 21. The cleaning blade 26 scrapes off and removes residual toner remaining on the surface of the photoconductor drum 21. Below the cleaning blade 26, a transport member 27 is disposed, which transports the toner (waste toner) scraped off by the cleaning blade 26 in the axial direction of the photoconductor drum 21. A description of transport of the waste toner is omitted.

Returns to FIG. 1, the LED heads 5K, 5C, 5M, and 5Y are disposed above and opposed to the photoconductor drums 21K, 21C, 21M, and 21Y of the image forming units 2K, 2C, 2M, and 2Y. The LED heads 5K, 5C, 5M, and 5Y each have a light emitting diode (LED) and a lens array, and form an image of light emitted from LED on the surface of the photoconductor drums 21K, 21C, 21M, and 21Y.

The transfer unit 4 is disposed below the image forming units 2K, 2C, 2M, and 2Y. The transfer unit 4 has a transfer belt 41 for electrostatically attracting and transporting the paper P, a drive roller 42 and a tension roller 43 over which the transfer belt 41 is extended, and four transfer rollers 40K, 40C, 40M, and 40Y which are disposed as transfer members to be opposed to the photoconductor drums 21K, 21C, 21M, and 21Y of the image forming units 2K, 2C, 2M, and 2Y.

The drive roller 42 is rotationally driven by a paper transport motor 109 (FIG. 3), and the transfer belt 41 is moved in the direction indicated by an arrow C. The tension roller 43 applies a predetermined tension to transfer belt 41.

The transfer belt 41 attracts the paper P on the surface, is moved by the rotation of the drive roller 42, and transports the paper P along the image forming units 2K, 2C, 2M, and 2Y. The transfer belt 41 is made of materials such as polyamide-imide or polyamide, and carbon is added to the materials to obtain conductivity and mechanical strength.

The transfer rollers 40K, 40C, 40M, and 40Y are in pressure contact with the photoconductor drums 21K, 21C, 21M, and 21Y via the transfer belt 41. A transfer voltage for transferring toner images formed on the surfaces of the photoconductor drums 21K, 21C, 21M, and 21Y is applied to the transfer rollers 40K, 40C, 40M, and 40Y.

The fixing unit 7 is disposed on the downstream side (the left side in FIG. 1) of the image forming units 2K, 2C, 2M, and 2Y in the transport direction of the paper P. The fixing unit 7 includes a heating roller 7a, a pressure roller 7b, and a thermistor 7c.

The heating roller 7a is a roller such that a heat-resistant elastic layer of silicone rubber is provided around a hollow cylinder-shaped core metal made of aluminum, and the surface of the heat-resistant elastic layer is covered with a tetrafluoroethylene-perfluoroalkyl vinyl ether copolymer

(PFA) tube. For instance, a heater such as a halogen lamp is provided inwardly of the core metal of the heating roller 7a.

The pressure roller 7b is a roller such that a heat-resistant elastic layer of silicone rubber is provided on the surface of the aluminum core metal, and the surface of the heat-resistant elastic layer is covered with a PFA tube. A pressure-contact portion (fixing nip) is formed between the pressure roller 7b and the heating roller 7a.

The thermistor 7c is a detection unit for the surface temperature of the heating roller 7a, and is disposed in the vicinity of the heating roller 7a in a non-contact manner. The temperature information detected by the thermistor 7c is outputted to a fixing controller 106 (FIG. 3). The fixing controller 106 controls ON and OFF of the heater in the heating roller 7a based on the temperature information of the thermistor 7c, and maintains the surface temperature of the heating roller 7a at a predetermined temperature.

The discharge roller pair 63 discharges the paper P delivered from the fixing unit 7 to the outside of the image forming apparatus 1, and is driven by the paper transport motor 109 (FIG. 3). The upper cover of the image forming apparatus 1 is provided with a stacker unit for placing the paper P discharged by the discharge roller pair 63.

It is to be noted that the image forming units 2K, 2C, 2M, and 2Y and the toner cartridges 3Y, 3M, 3C, and 3K are replaceable units in the image forming apparatus 1. Thus, when component parts deteriorate, or when toner is consumed, the image forming units 2K, 2C, 2M, and 2Y and the toner cartridges 3Y, 3M, 3C, and 3K can be replaced.

<Control System of Image Forming Apparatus>

Next, the control system of the image forming apparatus 1 will be described. FIG. 3 is a block diagram illustrating the principal unit of the control system of the image forming apparatus 1. As illustrated in FIG. 3, the image forming apparatus 1 has a controller 11, an interface controller 12, a receiving memory 13, an image data editing memory 14, an operation unit 15, and a sensor group 16.

The controller 11 includes a microprocessor, a ROM, a RAM, an input/output port, and a timer. The controller 11 receives print data and control commands from a higher-level device such as a personal computer, and performs a printing operation by controlling the entire sequence of the image forming apparatus 1.

The controller 11 has a dot counter 17, a drum counter 18, and a calculation unit 19. The dot counter 17 counts the number of dots necessary for printing based on the image data of the image data editing memory 14. The drum counter 18 counts the number of rotations of the photoconductor drum 21 which is rotated during a printing operation. The calculation unit 19 performs calculation based on information such as a temperature inputted from the sensor group 16, and the number of rotations counted by the drum counter 18.

The receiving memory 13 temporarily records the print data inputted from a higher-level device via the interface controller 12. The image data editing memory 14 receives the print data recorded on the receiving memory 13, and generates image data (that is, image data) by performing editing processing on the print data, and records the image data.

The operation unit 15 has a display (for instance, an LED) that displays the state of the image forming apparatus 1, and a switch and a display screen for inputting an instruction to the image forming apparatus 1 by an operator. The sensor group 16 includes various sensors for monitoring the operating state of the image forming apparatus 1, for instance, a paper position sensor that detects the position of the paper P,

a temperature-and-humidity sensor that detects temperature and humidity around the image forming apparatus 1, and a concentration sensor that detects the concentration of an image.

5 The image forming apparatus 1 further has a charging roller power source 101, a developing roller power source 102, a supply roller power source 103, a transfer roller power source 104, a head drive controller 105, a fixing controller 106, a transport motor controller 107, a drive controller 108, a paper transport motor 109, and a drive motor 110.

The charging roller power source 101 applies a charging voltage to the charging roller 22, the charging voltage for uniformly charging the surface of the photoconductor drum 21. The developing roller power source 102 applies a developing voltage to the developing roller 23, the developing voltage for causing toner to adhere to an electrostatic latent image of the photoconductor drum 21. The supply roller power source 103 applies a supply voltage to the supply roller 25, the supply voltage for supplying toner to the developing roller 23. The transfer roller power source 104 applies a transfer voltage to the transfer roller 40, the transfer voltage for transferring toner of the photoconductor drum 21 to the paper P.

15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9

The shaft 25b is made of metal having rigidity and conductivity, such as iron, copper, brass, stainless steel, aluminum, or nickel. However, the shaft 25b may be made of materials other than metal as long as the materials have rigidity and conductivity. For instance, the shaft 25b may be made of a resin molded article or ceramics in which conductive particles are distributed.

The shape of the shaft 25b may be an axial shape or a hollow pipe shape. At an end of the shaft 25b, a level difference 25c for mounting a gear may be formed or a pin hole or the like may be formed. At an end of the shaft 25b, a bearing having a diameter smaller the diameter of the central portion (that is, the portion surrounded by the conductive foam layer 25a) may be formed.

The outer diameter of the conductive foam layer 25a is nearly constant in the axial direction. However, the conductive foam layer 25a may have a crown shape or a tapered shape in which the outer diameter is smaller at a position closer to the axial end of the supply roller 25, or a shape in which the diameters at both ends are different.

The conductive foam layer 25a has air cells (cells) 201 which are open to the surface 200. The air cells 201 are closed air cells (closed cells) which are not continuous. The sizes of the air cells 201 are 200 to 300  $\mu\text{m}$ , for instance. The Asker F hardness of the conductive foam layer 25a is 30 degrees greater than and 50 degrees or less. Also, the stress decay of the conductive foam layer 25a is 25% or less, and the residual strain is 100  $\mu\text{m}$  or less.

The rubber material, of which the conductive foam layer 25a is made, contains silicone rubber as a main component. The main component indicates a component that accounts for 50% by weight or greater of the entirety. Also, silicone rubber may be denatured silicone rubber.

As an accessory component (component other than the main component), the rubber material, of which the conductive foam layer 25a is made, may contain crude rubber, nitrile rubber, ethylene-propylene rubber, ethylene propylene diene rubber (EPDM), styrene butadiene rubber, acrylonitrile-butadiene rubber, butadiene rubber, polyisoprene rubber, acrylic rubber, chloroprene rubber, butyl rubber, epichlorohydrin rubber, urethane rubber, fluoro-rubber, or polyether rubber. Also, the rubber material may contain elastomer such as polyurethane, polystyrene, polybutadiene block polymer, polyolefin, polyethylene, chlorinated polyethylene, ethylene-vinyl acetate copolymer. Also, one type or two or more types of these materials may be combined.

Although these rubber materials can be arbitrarily selected from a millable type or a liquid type, a rubber material of a millable type (in other words, a rubber material which has high viscosity and allows roll forming) is desirable.

Next, the manufacturing process of the supply roller 25 will be described. FIG. 5 is a flowchart illustrating the manufacturing process of the supply roller 25. First, a filler, a blowing agent, and a cross-linking agent are added to the above-described rubber material (step S101).

The filler includes a reinforcing filler and a conductive filler. For instance, silica (fumed silica or precipitated silica), or reinforcing carbon black may be used as the reinforcing filler. For instance, conductive carbon black, powder of metal such as nickel, aluminum, copper, a metal oxide such as zinc oxide, or barium sulfate, titanium oxide, or potassium titanate which is coated with tin oxide may be used as the conductive filler. Here, titanium, reinforcing carbon black, and conductive carbon black are used as the filler.

An azo compound-based blowing agent is used as the foaming agent. However, instead of an azo compound-based

blowing agent, bicarbonate-based, isocyanate-based, nitrite salt, hydrazine derivative, or azide compound-based blowing agent may be used.

A peroxide and a sulfur-based vulcanizing agent are used as the cross-linking agent (vulcanizing agent). However, instead of these, hydrogen siloxane in the presence of a platinum catalyst, or an isocyanate agent may be used.

Like this, a rubber material with a filler, a blowing agent, and a cross-linking agent added is mixed, and kneaded using 10 a pressure kneader or a mixing roll (step S102).

The kneaded material (rubber compound) is filled in an extruder, and is extruded to the surrounding of the shaft 25b and shaped (step S103). Consequently, a cylindrical rubber compound is shaped on the surface of the shaft 25b. Hereinafter, the shaft 25b in which the rubber compound is 15 formed on the surface is referred to as the roller body.

Next, thus shaped roller body is set in a heating furnace, and is heated to a temperature (for instance, approximately 150 to 160° C.) necessary for vulcanizing rubber (step 20 S104). In this step (primary vulcanization step), although vulcanization of rubber proceeds, no foam is produced.

After the primary vulcanization step, pre-vulcanization step (step S105) for foaming is performed. In the pre-vulcanization step, the roller body is heated at a temperature 25 higher than the temperature in the above-mentioned primary vulcanization step. FIG. 6 is a graph illustrating a temperature rise curve in the pre-vulcanization step and the secondary vulcanization step (described below), the vertical axis indicates temperature, and the horizontal axis indicates time.

The pre-vulcanization step corresponds to the time period t0 to t1 illustrated in FIG. 6. In the pre-vulcanization step, the temperature rises to a temperature T2 which is the peak temperature, then falls to a temperature T1 lower than the temperature T2. The temperatures T1, T2 are each higher 30 than the heating temperature (approximately 150 to 160° C.) in the primary vulcanization step. Thus, foaming occurs, and air cells are formed, thus vulcanization of rubber proceeds.

After the pre-vulcanization step, the roller body is taken out from the heating furnace, and the outer circumference of 40 the foam layer of the roller body is roughly polished (step S106). Here, a range with several millimeters of thickness of the outer circumference (surface) of the foam layer is removed by rough polishing. In the above-described primary vulcanization step and pre-vulcanization step, a skin layer 45 having small air cells is formed on the outer circumference of the foam layer, and the skin layer is removed by rough polishing.

Subsequently, the roughly-polished roller body is set in the heating furnace, and the secondary vulcanization step (step S107) is performed. The secondary vulcanization step corresponds to the time period t1 to t2 illustrated in FIG. 6. In the secondary vulcanization step, the roller body is heated to the temperature T1 mentioned above. Consequently, air 50 cells are further formed, and vulcanization of rubber proceeds. It is to be noted that before time t1, there is practically a temperature rise process after the roller body is set in the heating furnace.

Since a skin layer is removed beforehand in the secondary vulcanization step, unbalance (distortion) of the cross-linking state of the rubber can be reduced, and air cells can be 60 uniformly formed (that is, with a uniform size over the entire surface of the foam layer). Also, in the secondary vulcanization step, low-molecular siloxane derived from silicone is removed by volatilization, and since a skin layer has been 65 removed from the surface of the foam layer as described above, the low-molecular siloxane can be effectively removed.

After the secondary vulcanization step, finish machining is performed on the surface of the foam layer of the roller body, and a predetermined outer diameter is obtained (step S108). Consequently, the supply roller 25 is formed, in which the conductive foam layer 25a is formed on the surface of the shaft 25b.

<Functional Effect>

Next, the functional effect of the supply roller 25 will be described. As described above, the conductive foam layer 25a of the supply roller 25 contains silicone rubber as a main component. A general conductive foam layer containing urethane rubber as a main component has continuous air cells (in other words, the air cells are connected). In contrast, the conductive foam layer 25a containing silicone rubber as a main component has closed cells (in other words, the air cells are independent from each other).

In the case of a conductive foam layer having continuous air cells, toner can enter deep inside the air cells, and thus the toner may get clogged in the air cells. Therefore, as the number of sheets printed by the image forming apparatus 1 increases, the amount of toner clogged in the air cells increases, and as a result, the hardness and the electric resistance of the conductive foam layer increase, and image unevenness (blur) due to insufficient toner supply occurs.

In contrast, in the case of a conductive foam layer having closed air cells, toner does not enter deep inside the air cells, and thus clogging of toner in the air cells is unlikely to occur. Therefore, even when the number of sheets printed by the image forming apparatus 1 increases, the hardness and the electric resistance of the conductive foam layer has a low increase, and the occurrence of image unevenness (blur) is also suppressed.

Also, the stress decay of the conductive foam layer 25a of the supply roller 25 is 25% or less, and the residual strain is 100  $\mu\text{m}$  or less. The conductive foam layer 25a has a configuration in which permanent strain is unlikely to occur.

Therefore, even when the conductive foam layer 25a of the supply roller 25 is left unoperated for a long period of time with depressed by the developing roller 23, and a depressed area is formed at the depressed portion, if a pressing pressure is released, the shape of the conductive foam layer 25a is likely to be restored. Therefore, even when printing is performed after a long period of time of non-operation, insufficient toner supply is unlikely to occur, and the occurrence of image unevenness can be suppressed.

Also, the conductive foam layer 25a containing silicone rubber as main component has a longer life than a general conductive foam layer containing urethane rubber as a main component. Therefore, the supply roller 25 needs to be replaced with a less frequency.

Also, as described above, in the vulcanization step of the supply roller 25, the conductive foam layer 25a is caused to foam in the pre-vulcanization step, and a skin layer on the surface is removed, and the secondary vulcanization steps is performed anew. Thus, air cells can be uniformly formed.

Also, in the secondary vulcanization step, removal of the low-molecular siloxane by volatilization is not prevented by a skin layer, and thus the low-molecular siloxane can be effectively removed.

<Operation of Image Forming Apparatus>

Next, the operation of the image forming apparatus 1 will be described with reference to FIGS. 1 and 3. The image forming units 2K, 2C, 2M, and 2Y of the image forming apparatus 1 receive supply of black, cyan, magenta, and yellow toner from the toner cartridges 3K, 3C, 3M, and 3Y, and are in a printable state.

When the controller 11 of the image forming apparatus 1 receives print data and control commands from a higher-level device such as a personal computer via the interface controller 12, the controller 11 starts a printing operation (image forming operation).

The transport motor controller 107 drives the paper transport motor 109 by an instruction of the controller 11, and the paper P in the paper feed cassette 60 is delivered in the direction indicated by the arrow A by the pickup roller 61. Furthermore, the paper P is delivered in the direction indicated by the arrow B by the transport roller pair 62. Also, the drive roller 42 rotates, and moves the transfer belt 41 in the direction indicated by the arrow C.

The transfer belt 41 attracts, holds and transports the paper P so that the paper P is passed through the image forming units 2K, 2C, 2M, and 2Y.

Also, the drive controller 108 drives the drive motor 110 by an instruction of the controller 11, and rotates the photoconductor drums 21K, 21C, 21M, and 21Y. The rotation of the drive motor 110 is also transmitted to the developing rollers 23K, 23C, 23M, and 23Y and the supply rollers 25K, 25C, 25M, and 25Y, and the developing rollers 23K, 23C, 23M, and 23Y and the supply rollers 25K, 25C, 25M, and 25Y are also rotated.

In the image forming units 2K, 2C, 2M, and 2Y, the charging rollers 22K, 22C, 22M, and 22Y each receive application of a charging voltage (a bias voltage having the same polarity as that of toner) by the charging roller power source 101, and uniformly charge the surface of each of the photoconductor drums 21K, 21C, 21M, and 21Y.

The LED heads 5K, 5C, 5M, and 5Y are driven by the head drive controller 105, and expose the surfaces of the photoconductor drums 21K, 21C, 21M, and 21Y to light based on the image data of each color, and form an electrostatic latent image.

The developing rollers 23K, 23C, 23M, and 23Y each receive application of a developing voltage (a bias voltage having the same polarity as or the reverse polarity to that of toner) by the developing roller power source 102, and charge the toner adhering to the surfaces.

The developing blades 24K, 24C, 24M, and 24Y are pressed against the developing rollers 23K, 23C, 23M, and 23Y, and regulate the thickness of each toner layer on the surfaces of the developing rollers 23K, 23C, 23M, and 23Y. It is to be noted that a bias voltage (blade voltage) may be applied to the developing blades 24K, 24C, 24M, and 24Y by the developing roller power source 102 or the supply roller power source 103.

The supply rollers 25K, 25C, 25M, and 25Y each receive application of a supply voltage (a bias voltage having the same polarity as or the reverse polarity to that of toner) by the supply roller power source 103, and supply the toner supplied from the toner cartridges 3K, 3M, 3Y, and 3C to the developing rollers 23K, 23C, 23M, and 23Y.

Furthermore, the supply rollers 25K, 25C, 25M, and 25Y have a function of charging toner by contact friction with the developing rollers 23K, 23C, 23M, and 23Y as well as a function of collecting the toner not used for development from the developing rollers 23K, 23C, 23M, and 23Y.

The cleaning blades 26K, 26C, 26M, and 26Y scrape off and remove the residual toner remaining on the surfaces of the photoconductor drums 21K, 21C, 21M, and 21Y. The cleaning blades 26K, 26C, 26M, and 26Y also scrape off and remove adhering materials which have adhered to the surface of photoconductor drums 21K, 21C, 21M, and 21Y from the transfer belt 41 although the amount of adhering materials is very small in quantity.

## 11

The transport members 27K, 27C, 27M, and 27Y transport the toner (waste toner) and the adhering materials scraped off from the photoconductor drums 21K, 21C, 21M, and 21Y by the cleaning blades 26K, 26C, 26M, and 26Y.

The transfer rollers 40K, 40C, 40M, and 40Y of the transfer unit 4 each receive application of a transfer voltage (a bias voltage the reverse polarity to that of toner) by the transfer roller power source 104, and transfer a toner image of each color from the photoconductor drums 21K, 21C, 21M, and 21Y to the paper P.

The paper P, to which a toner image of each color has been transferred in this manner, is further transported by the transfer belt 41, and arrives at the fixing unit 7. In the fixing unit 7, the fixing controller 106 controls the heater of the heating roller 7a based on the surface temperature of the heating roller 7a detected by the thermistor 7c, and maintains the surface temperature of the heating roller 7a at a predetermined temperature. The paper P with a toner image transferred is passed through the pressure-contact portion (fixing nip) between the heating roller 7a and the pressure roller 7b, and heat and pressure are thereby applied onto the toner image which is fixed to the paper P.

The paper P with the toner image fixed is transported by the discharge roller pair 63 which is rotated by the paper transport motor 109, and is discharged to the outside of the image forming apparatus 1.

<Print Test>

Next, a print test for verifying the functional effect of the supply roller 25 will be described. First, in the manufac-

## 12

of 13 mm are supported by a pair of supports 81. A cylindrical gauge head 80 having a length of 50 mm and an outer diameter of 16 mm is pressed against the axial center of the outer circumferential surface of the conductive foam layer 25a of the supply roller 25.

In this state, the supply roller 25 is pressed by the gauge head 80 (compression step 1 illustrated in FIG. 8) so that a displacement amount (d1) is 1 mm at a displacement speed of 10 mm/min. In this state, the gauge head 80 remains at rest for 1 hour (stress decay step 2 illustrated in FIG. 8). Subsequently, the gauge head 80 is returned to the original position at a displacement speed of 10 mm/min (decompression step 3 illustrated in FIG. 8). The stress decay and the residual strain can be determined from the hysteresis loop illustrated in FIG. 8.

Specifically, in the hysteresis loop of FIG. 8, let Pmax be the maximum stress at the completion time of the compression step 1, Pmin be the stress (stress at the time of decay) at the completion time of the stress decay step 2, and dx be the displacement amount when the compression stress is 0 in the decompression step 3. The stress decay can be determined by  $(P_{max} - P_{min})/P_{max} \times 100\%$ . Also, the residual strain, that is, the displacement amount at the time of release of stress is dx (μm).

The hysteresis loop of FIG. 8 is produced for each of all supply rollers 25 in Examples 1 to 3 and Comparative Examples 1 to 3, and the stress decay and the residual strain of the conductive foam layer 25a are measured. The result is illustrated in Table 1.

TABLE 1

| Supply Roller         | Stress Decay (%) | Residual Strain (μm) | Air Cell state   | Asker F Hardness | Presence of Horizontal White Strip | Others     |
|-----------------------|------------------|----------------------|------------------|------------------|------------------------------------|------------|
| Comparative Example 1 | 37               | 235                  | Closed Cells     | 50               | Present                            | —          |
| Comparative Example 2 | 30               | 131                  | Closed Cells     | 55               | Partially Present                  | —          |
| Comparative Example 3 | 24               | 94                   | Continuous Cells | 30               | Absent                             | Image Blur |
| Example 1             | 23               | 98                   | Closed Cells     | 30               | Absent                             | —          |
| Example 2             | 20               | 87                   | Closed Cells     | 40               | Absent                             | —          |
| Example 3             | 18               | 81                   | Closed Cells     | 50               | Absent                             | —          |

ing process illustrated in FIG. 5, the time t1 and the temperature T1 (FIG. 6) in the pre-vulcanization step are made different, and thus the supply rollers 25 in Examples 1, 2, 3 and Comparative Examples 1, 2, 3 are produced with different stress decays and residual strains.

In Examples 1, 2, 3 and Comparative Examples 1, 2, silicone rubber is used as the rubber material, and in Comparative Example 3, urethane rubber is used as the rubber material. In each of Examples 1 to 3 and Comparative Examples 1 to 3, cyan, reinforcing carbon black, and conductive carbon black are used as the filler, and an azo compound-based blowing agent is used as the foaming agent, and a peroxide and a sulfur-based vulcanizing agent are used as the cross-linking agent.

FIG. 7 is a schematic illustration depicting a method of measuring hysteresis characteristics for determining stress decay and residual strain. FIG. 8 is a graph illustrating a hysteresis loop (stress-strain curve). To measure hysteresis characteristics, mechanical displacement meter "5543A" manufactured by Intron corporation is used. As illustrated in FIG. 7, in the mechanical displacement meter, both ends of the shaft 25b of the supply roller 25 having an outer diameter

45 Table 1 further illustrates an air cell state (continuous cells or closed cells) and the Asker F hardness of the conductive foam layer 25a for each of the supply rollers 25 in Examples 1 to 3 and Comparative Examples 1 to 3.

50 Next, each of the supply rollers 25 in Examples 1 to 3 and Comparative Examples 1 to 3 is mounted in an image forming unit 2C of the image forming apparatus 1 (FIG. 1), and is left for one month in contact with the developing roller 23 in an environment with a temperature of 47°C. and a relative humidity of 66%. After each supply roller 25 is left 55 for one month, a print test is conducted by the image forming apparatus 1.

60 "Color LED printer C542dnw" manufactured by OKI data Co., Ltd. is used as the image forming apparatus 1, and only the image forming unit 2C for cyan is mounted out of four image forming units 2K, 2C, 2M, and 2Y. "Xerox 4200 LT 20lb New92" (letter size) manufactured by Fuji Xerox Co., Ltd. is used as the paper P.

65 As a print pattern, a solid pattern (solid image) of cyan with a print duty of 100% is used. Intermittent printing of one page is performed with single-sided printing. Also, the number of printed sheets is three, and the last sheet is visually observed.

FIG. 9 is a schematic illustration depicting an example of image unevenness which occurs in the print pattern. The direction indicated by the arrow B in FIG. 9 is the transport direction of the paper P. When a typical supply roller is left in contact with the developing roller for a long period of time, and subsequently, printing is performed, toner supply is insufficient at a depressed area formed in the conductive foam layer of the supply roller, and thus white strips of uneven image (that is, horizontal white strips) occur as indicated by symbol E in FIG. 9. The horizontal white strips extend with a width of several mm in the axial direction of the photoconductor drum (in other words, in the axial direction of the developing roller).

The pattern printed with image forming device 1 incorporating A pattern printed by the image forming apparatus 1 which is incorporated with any supply roller 25 in Comparative Examples 1 to 3 and Examples 1 to 3 is visually observed, and the presence of a horizontal white strip is determined. The result of determination of the presence of a horizontal white strip is presented in the table 1 above.

As illustrated in Table 1, in Comparative Examples 1, 2 in which the stress decay is 30% or greater and the residual strain is 100  $\mu\text{m}$  or greater in the conductive foam layer 25a, occurrence of a horizontal white strip is observed. Also, in Comparative Example 3 in which urethane rubber is the main component of the conductive foam layer 25a, the stress decay is 24%, and the residual strain is 94  $\mu\text{m}$  (that is, the characteristics in which permanent strain is unlikely to occur), and occurrence of a horizontal white strip is not observed. However, occurrence of image blur is observed in a printed image.

In contrast, in Examples 1, 2, 3 in which silicone rubber is the main component of the conductive foam layer 25a, the stress decay is 25% or less (specifically, 23%, 20%, 18%, respectively), and the residual strain is 100  $\mu\text{m}$  or less (specifically, 98  $\mu\text{m}$ , 87  $\mu\text{m}$ , 81  $\mu\text{m}$ , respectively), occurrence of a horizontal white strip is not observed. Also occurrence of image blur is not observed.

This is probably because when the stress decay is 25% or less and the residual strain is 100  $\mu\text{m}$  or less in the conductive foam layer 25a, even when the conductive foam layer 25a is left for a long period of time with depressed by the developing roller 23, permanent strain is unlikely to occur (in other words, a depressed area formed in the conductive foam layer 25a is likely to be restored to the original shape), and therefore, occurrence of a horizontal white strip is suppressed.

Also, when the main component of the conductive foam layer 25a is urethane rubber, continuous air cells are formed, and thus toner is likely to get clogged in the continuous air cells. As the number of printed sheets increases, the hardness and the electric resistance of the conductive foam layer 25a increase, and image blur is caused. In contrast, when the main component of the conductive foam layer 25a is silicone rubber, closed air cells are formed, and thus toner is unlikely to get clogged, and as a result, occurrence of image blur is probably suppressed.

Also, each conductive foam layer 25a in Examples 1 to 3 has the Asker F hardness of 30 or greater and 50 or less. Since each conductive foam layer 25a in Examples 1 to 3 is relatively flexible like this, a depressed area formed in the conductive foam layer 25a is likely to be restored to the original shape, and as a result, an image unevenness suppression effect is probably enhanced.

## &lt;Effect&gt;

As described above, according to an embodiment, the supply roller 25 (developer supply member) has the conductive foam layer 25a containing silicone rubber as a main component,

the stress decay is 25% or less and the residual strain is 100  $\mu\text{m}$  or less in the conductive foam layer 25a, even when printing is performed after the conductive foam layer 25a is left unoperated for a long period of time with depressed by the developing roller 23, occurrence of image unevenness can be suppressed. Also, since closed air cells are formed, toner is unlikely to get clogged, and occurrence of image blur can be suppressed. Consequently, image quality can be improved.

Also, the conductive foam layer 25a containing silicone rubber as a main component has a longer life than any conductive foam layer containing urethane rubber as a main component. Therefore, the supply roller 25 needs to be replaced with a less frequency.

Also, since the supply roller 25 has no skin layer (which is removed in a rough polishing process), unbalance (distortion) of the cross-linking state of the rubber can be reduced, and air cells can be uniformly formed. Also, removal of the low-molecular siloxane by volatilization is not prevented by a skin layer, and thus the low-molecular siloxane can be effectively removed.

## Modification

FIG. 10 is a flowchart illustrating a modification of the manufacturing process of the supply roller 25. In the manufacturing process illustrated in FIG. 5, after a rubber compound is shaped on the shaft 25b (step S103), the primary vulcanization step (step S104) is performed. However, as illustrated in FIG. 10, a rubber compound may be molded into a tube shape by an extruder (step S103A), and after the tube is put on the shaft 25b (step S103B), the primary vulcanization step (step S104) may be performed. Other steps S101, 102, 104 to 108 are as described with reference to FIG. 5.

Although a printer using the electrophotography has been described in an embodiment, the present invention is not limited to this, and is applicable to, for instance, a facsimile, a copying machine, a multi-function peripheral (MFT) using the electrophotography.

Although a preferable embodiment of the present invention has been specifically described above, the present invention is not limited to the embodiment, and various improvements and modifications may be made in a range not departing from the essence of the present invention. The invention includes other embodiments in addition to the above-described embodiments without departing from the spirit of the invention. The embodiments are to be considered in all respects as illustrative, and not restrictive. The scope of the invention is indicated by the appended claims rather than by the foregoing description. Hence, all configurations including the meaning and range within equivalent arrangements of the claims are intended to be embraced in the invention.

The invention claimed is:

1. A developer supply member comprising:  
a shaft with conductivity; and  
a conductive foam layer that is formed on a surface of the shaft and that contains silicone rubber as a main component, and includes a stress decay of 25% or less and a residual strain of 100  $\mu\text{m}$  or less.
2. The developer supply member according to claim 1, wherein Asker F hardness of the conductive foam layer is 30 degrees or greater and 50 degrees or less.

**15**

3. The developer supply member according to claim 1, wherein the conductive foam layer includes closed air cells. 5
4. The developer supply member according to claim 3, wherein the air cells contain air cells with a diameter of 200 to 300  $\mu\text{m}$ . 10
5. The developer supply member according to claim 1, wherein the conductive foam layer further contains a filler, a cross-linking agent, and a blowing agent. 15
6. The developer supply member according to claim 1, wherein in the conductive foam layer, the silicone rubber accounts for 50% by weight or greater of a rubber component contained in the conductive foam layer. 20
7. An image forming unit comprising:  
a developer carrier that supplies a developer to a latent image formed on an image carrier to form a developer image on the image carrier; and  
the developer supply member according to claim 1 that is disposed in contact with the developer carrier. 25
8. The image forming unit according to claim 7, wherein the developer supply member is rotated in such a direction that movement directions of surfaces in contact with each other of the developer supply member and the developer carrier are opposite to each other. 30
9. An image forming unit comprising:  
an image carrier that carries a latent image thereon;  
a developer carrier that supplies a developer to the latent image on the image carrier to form a developer image; and  
the developer supply member according to claim 1 that is disposed in contact with the developer carrier and that supplies the developer to the developer carrier. 35
10. An image forming apparatus comprising:  
the image forming unit according to claim 9;  
a transfer unit that transfers the developer image from the image carrier onto a medium; and  
a fixing unit that fixes the developer image to the medium. 35

**16**

11. A developer supply member comprising:  
a shaft with conductivity; and  
a conductive foam layer formed on a surface of the shaft, wherein the conductive foam layer is formed by performing a primary vulcanization, pre-vulcanization, surface polishing and a secondary vulcanization on a rubber compound which contains silicone rubber as a main component and to which a blowing agent and a vulcanizing agent are added. 10
12. The developer supply member according to claim 11, wherein a surface skin layer of the conductive foam layer is removed by the surface polishing. 15
13. The developer supply member according to claim 11, wherein a temperature of the pre-vulcanization is higher than a temperature of the primary vulcanization. 20
14. An image forming unit comprising:  
a developer carrier that supplies a developer to a latent image on an image carrier to form a developer image on the image carrier; and  
the developer supply member according to claim 11 that is disposed in contact with the developer carrier and that supplies the developer to the developer carrier. 25
15. The image forming unit according to claim 14, wherein the developer supply member is rotated in such a direction that movement directions of surfaces in contact with each other of the developer supply member and the developer carrier are opposite to each other. 30
16. An image forming unit comprising:  
an image carrier that carries a latent image thereon;  
a developer carrier that supplies a developer to the latent image on the image carrier to form a developer image; and  
the developer supply member according to claim 11 that is disposed in contact with the developer carrier and that supplies the developer to the developer carrier. 35
17. An image forming apparatus comprising:  
the image forming unit according to claim 16;  
a transfer unit that transfers the developer image from the image carrier onto a medium; and  
a fixing unit that fixes the developer image to the medium. 40

\* \* \* \* \*